

## UNITED STATES PATENT OFFICE.

VICTOR NOAK HYBINETTE, OF JACKSON, MICHIGAN, ASSIGNOR TO HYBINETTE PATENTS CORPORATION, OF JACKSON, MICHIGAN.

## PLASTIC LIGHT ALUMINUM ALLOY AND PROCESS OF PRODUCING SAME.

No Drawing.

Application filed July 11, 1927. Serial No. 205,028.

My invention relates to further development of the process and product described in a now pending U. S. patent application, Ser. No. 165,246, filed Feb. 1, 1927.

5 Said application described an alloy of about 95-97% aluminum, with small quantities of nickel, chromium, tungsten, molybdenum, manganese, iron, and zinc in variable proportions, to which is added a limited 10 amount of copper and magnesium, about 0.3-0.5% of each. The peculiar properties of this alloy are set forth in said application to be age-hardening at high temperature between fairly wide limits. Different predetermined 15 degrees of physical properties are to be obtained by adjusting composition and length of time and degree of temperature of aging.

The present application covers the results 20 of further research of the properties of this type of alloy.

I have found that this alloy may be worked after quenching from about 900-950° F. both before and after aging, and particularly 25 by alternating periods of aging and working, and that for best results it should be somewhat modified in composition.

By such work rolling or forging the property of not hardening under work is more 30 and more developed until a nearly perfect plastic alloy is obtained. In this way I have produced sheets with over 50,000 lbs. yield point, which may be bent over flat and the bend hammered out to an edge without sign 35 of cracking. That such metal is valuable for rivets, piston rods, etc., as well as for spinning and forming, is evident.

I proceed with the production of this alloy very much as described in the above referred 40 to application. For the highest degree of plasticity I reduce the hardening elements such as manganese, or eliminate them altogether. Iron in the presence of nickel seems not to be at all detrimental. In fact, if no 45 iron is present the alloy must contain more of the other heavy metals to produce the same strength. In practice it is almost impossible to produce such alloy without about 0.5% iron. Silicon hardens the alloy and reduces 50 plasticity. So does magnesium and copper. I can get along with as little as 0.10-0.15% magnesium if the copper is high. All raw materials contain silicon, and I must therefore select low silicon raw material so as not

to have over 0.5% silicon in my final product. 55 When silicon is low I may use more magnesium. My preferred composition contains about 1.5-2% of a mixture of nickel with chromium and/or tungsten, molybdenum, manganese, iron and zinc. Where the nickel 60 is predominating, I may use 1% nickel and 0.5% chromium, or 1% nickel and 0.1-0.2% each of all the other metals, or I may use about 2% nickel only.

The presence of the chromium group of 65 metals is not all important in this case, because I obtain all necessary strength by aging and working. For non-corroding or non-tarnishing, it is important to leave them in. The main thing is that I have nickel and some 70 other metal because of all heavy metals, nickel seems to be the least harmful when it comes to producing an alloy of high plasticity, but nickel alone will not give an ultimate strength of much over 40,000 lbs. Zinc up to 75 2% does not seem to have any harmful influence. With these heavy metals I introduce the copper, magnesium and silicon above referred to, so that my standard alloy will analyze about as follows:

|                       |            |                      |
|-----------------------|------------|----------------------|
| Nickel                | 0.75-2.00% | Total about 1.5-2.5% |
| Chromium              | 0- .50%    |                      |
| Tungsten              | 0- .50%    |                      |
| Molybdenum            | 0- .50%    |                      |
| Manganese             | 0- .50%    |                      |
| Iron (as impurity)    | 0.30- .60% |                      |
| Zinc                  | 0- 2.00%   |                      |
| Copper                | 0.20- .50% |                      |
| Magnesium             | 0.10- .50% | Total about 1%       |
| Silicon (as impurity) | 0.2- .50%  |                      |
| Aluminum about        | 96-97.00%  |                      |

80

85

The compounding of the alloy is well understood by those conversant with the art, 90 and is fully described in U. S. Patent #1,579,481 of April 6, 1926. The main idea is that I cut down all hardening elements to a minimum.

The alloy so produced is forged or rolled 95 hot and cold in the usual way with or without intermediate annealing. It is then heated to about 900-950° F. and quenched in water.

If this alloy is aged for 12-24 hours at temperature below 300° F. and if it contains less 100 than 0.50% copper and magnesium combined, and less than 0.20% of magnesium, a slight increase in elongation is the only change observed. At 310° F. the alloy containing 0.10% magnesium and 0.50% copper becomes 105 more ductile, but the ultimate strength and yield point remain unchanged. It seems to require 0.25% of each to obtain a commer-

cially valuable heat treatment, although for some purposes the increased elongation may be desirable.

The quenched standard alloy has about 5 16,000 lbs. yield and 26,000 lbs. ultimate strength with about 12-15% elongation. Aged at 310° F. for 24 hours it will show about 35,000 lbs. yield point and 42,000 lbs. ultimate strength, with 6-8% elongation. It 10 will not bend over without cracking.

If it is rolled to a reduction of 20-30% in thickness after quenching, or if it is rolled the same way after aging, it gives about the same result of increased strength to about 48,000 15 lbs. yield point and ultimate elongation 2-3%, but a better bending quality. It is more plastic.

If it is rolled both before and after aging, and then rolled again and aged again, each 20 rolling reduction being 20-30%, and each period of aging lasting about 12-24 hours at 300-400° F., it obtains the maximum of plasticity, and strength above referred to.

The final strength is a function of the total 25 reduction after quenching and also, in a lesser degree perhaps, of the composition of the alloy, but the degree of plasticity is depending mainly upon the number of steps of working and aging.

If the desired plasticity is not obtained, it 30 is an indication that some of the additions have been made in too large quantity. I have rolled such finished product down from a thickness of 0.030" to 0.003", a reduction of 35 90% without any sign of increased hardness.

At the same time the yield point and ultimate strength remain stationary at 40,000-55,000 lbs. That such alloy has a remarkable resistance to fatigue, is natural, because fatigue is nothing but hardening under work. Its perfect flowing quality makes it ideal for cold work, such as riveting. 40

When the alloy contains the chromium group metals it is remarkable for its non-tarnishing quality and resistance to corrosion. 45

It will thus be seen that my invention consists in alloying the aluminum with quantities below the maximum used in an alloy designed for hardness and great strength, and by 50 quenching and aging in combination with working, obtaining heretofore unheard-of qualities of plasticity and strength, which makes the product useful for certain purposes, where lightness, low fatigue, strength, 55 and non-corrodibility are needed.

I claim as my invention:

The process of producing a highly plastic, strong, light aluminum alloy which comprises first alloying the aluminum with less than 60 2½% of heavy metals and less than ½% of copper, and ½% of magnesium to make the resulting alloy only slightly responsive to heat treatment, and bringing out the strength and plasticity by working the metal after it is 65 quenched and before it is fully aged in intermittent periods of aging and working.

In testimony whereof I affix my signature.

VICTOR NOAK HYBINETTE.